# EUROPEAN PATENT SPECIFICATION

(11) **EP 3 348 712 B1**
(45) Date of publication and mention of the grant of the patent: **20.11.2019**
(21) Application number: 16898333.6
(22) Date of filing: 30.05.2016
(51) Int. Cl.: E01D 19/16, D07B 1/10, D07B 3/00, D07B 5/00

(54) **METHOD FOR MANUFACTURING HOT EXTRUDED POLYETHYLENE ZINC-ALUMINIUM ALLOY-PLATED STEEL WIRE HAULING CABLE**
VERFAHREN ZUR HERSTELLUNG EINES HEISSEXTRUDIERTEN, MIT EINER POLYETHYLEN-ZINK-ALUMINIUM-LEGIERUNG PLATTIERTEN STAHLDRAHTFÖRDERSEILS
PROCÉDÉ DE FABRICATION D'UN CÂBLE DE TRACTION À FILS D'ACIER PLAQUÉS D'UN ALLIAGE DE ZINC-ALUMINIUM, RECOUVERT DE POLYÉTHYLÈNE EXTRUDÉ À CHAUD

(30) Priority: 13.04.2016 CN 201610229109
(43) Date of publication of application: 18.07.2018
(73) Proprietor: Jiangsu Fasten Steel Cable Co., Ltd., Jiangyin Jiangsu 214445 (CN)
(72) Inventor: ZHAO, Jun, Jiangyin, Jiangsu, 214445 (CN); NING, Shiwei, Jiangyin, Jiangsu, 214445 (CN); XUE, Huajuan, Jiangyin, Jiangsu, 214445 (CN); ZHOU, Zhubing, Jiangyin, Jiangsu, 214445 (CN); WU, Qiong, Jiangyin, Jiangsu, 214445 (CN); QIANG, Qiang, Jiangyin, Jiangsu, 214445 (CN); HUANG, Kebin, Jiangyin Jiangsu, 214445 (CN); ZHU, Xiaoxiong, Jiangyin, Jiangsu, 214445 (CN); SHU, Weihong, Jiangyin, Jiangsu, 214445 (CN); WANG, Jin, Jiangyin, Jiangsu, 214445 (CN); LIANG, Zhongmei, Jiangyin, Jiangsu, 214445 (CN); ZHAI, Pengcheng, Jiangyin, Jiangsu, 214445 (CN)
(74) Representative: Huang, Liwei
(86) International application number: PCT/CN2016/083894
(87) International publication number: WO 2017/177518

(56) References cited:
- EP-A1- 0 855 471
- CN-A- 1 091 791
- CN-A- 1 672 906
- CN-A- 101 608 431
- CN-B- 101 949 130
- CN-U- 201 704 627
- CN-Y- 2 635 725
- DE-U1-202007 007 210
- JP-A- 2014 232 638
- Chitoshi Miki ET AL: "Full-size fatigue test of bridge cables", , 31 December 1992 (1992-12-31), XP055499829, DOI: 10.5169/seals-50695 Retrieved from the Internet: URL:https://www.e-periodica.ch/cntmng?pid= bse-re-003:1992:66::21 [retrieved on 2018-08-15]
- Manabu Ito: "Stay cable technology: overview", , 31 December 1999 (1999-12-31), XP055499827, Retrieved from the Internet: URL:https://www.e-periodica.ch/cntmng?pid= bse-re-003:1999:82::11 [retrieved on 2018-08-15]
- Anonymous: "EN 1993-1-11", , 1 January 2009 (2009-01-01), XP055499624, Retrieved from the Internet: URL:https://www.phd.eng.br/wp-content/uplo ads/2015/12/en.1993.1.11.2006.pdf [retrieved on 2018-08-14]
- Anonymous: "HD Stay Cable - Freysssinet", , 23 May 2013 (2013-05-23), XP055499638, Retrieved from the Internet: URL:https://freyssinet.co.uk/wp-content/up loads/2016/01/Freyssinet-HD-Stay-Cable.pdf [retrieved on 2018-08-14]
- Wandinger ET AL: "Technische Mechanik", , 23 July 2015 (2015-07-23), XP055492616, DOI: 10.1002/stab.201201503 Retrieved from the Internet: URL:https://web.archive.org/web/2015072319 3305if_/http://wandinger.userweb.mwn.de:80 /LA_TMET/v2_1.pdf [retrieved on 2018-07-16]
- Anonymous: "Hanging-Cable and Tied-Cable-BESTEN", , 15 August 2018 (2018-08-15), XP055499830, Retrieved from the Internet: URL:http://bestenchina.com/index.php?g=&m= Product&a=show&id=308 [retrieved on 2018-08-15]

## Description

The invention belongs to the technical field of bridge cable, and relates to a method for fabricating a steel wire cable comprising an extruded polyethylene and a zinc-aluminum alloy plating.

A cable-stayed bridge has one or more towers, from which cables support the bridge deck. The cable-stayed bridge features light structure and strong applicability, and is able to form different systems by varying the combination of bridge deck, cables, and towers according to different geologic environment and terrains. Due to the addition of the stay cables, a bending moment of a main girder is significantly decreased. Compared with large-span bridges of other systems, the uses of the steel and the concrete of the main girder in the cable-stayed bridge are relatively saved. Under the action of the pre-tension of the cable-stayed bridge, an internal force of the main girder can be adjusted to make the distribution thereof uniform and therefore acquire better economic effect. In addition, the main girder can be manufactured as a uniform girder, thus being convenient for manufacture and installation. A horizontal component force of the stay cable is equivalent to a pre-pressure applied to the main girder, which further improves the crack resistance of the girder (especially the concrete girder) and fully presents the performances of the materials.

The concept of cable-stayed bridge was originated from 17th century but not well developed due to condition restrictions at that time. In 1784, a German named CJLoscher built a 32 m-span wooden cable-stayed bridge in Friborg. The bridge adopts a support system formed by wooden tension rods connected to wooden towers and is the first truly cable-stayed bridge. After World War II, with the rebuild of the Europe and the developments in the modern mechanics theory and technologies, in order to seek the both economic and convenient bridge, the cable-stayed bridge attracted the attention of the public and was recognized to possess great advantages in a certain span range. The world's first modern cable-stayed bridge was the Stro msund Bridge built in 1955 in Sweden, and was a steel cable-stayed bridge having a span of 182.6 m across the Strom Strait, marking the beginning of modern cable-stayed bridges. In 1962, the world's first concrete cable-stayed bridge was built in Venezuela (with a main span of 135 meters). At that time, the cable-stayed bridge had gained rapid development. By the end of the twentieth century, the Norman Bridge, with a main span of 856 meters, had been built in France, and the Duo Luo Bridge, with a main span of 890 meters, had been built in Japan. Cables of all these bridges adopts hot galvanized stranded wire or steel wire.

With the quick development of the modern bridge, many sea-crossing bridges with ultra-long span will be built in the future, the stay cable of which is required to have long length, high accuracy, and long designed service life. However, the conventional galvanized steel wire cable is unable to meet the endurance requirement for the ultra-long span sea-crossing bridge.

Chitoshi Miki ET AL:"Full-size fatigue test of bridge cables" (1992) discloses on page 169 two stay cables, identified as HIAM SPWS-163 and New PWS-163, for example, a cable is made of semiparallel wires with HiAm sockets.

In view of the above-described problems, it is one objective of the invention to provide a method for fabricating a steel wire cable comprising an extruded polyethylene and a zinc-aluminum alloy plating. In which, steel wires are arranged according to an arrangement rule at a cross section of the steel wire cable; a length of the overall cable is controlled by a length of a central standard wire; a bunch of the steel wires comprising a zinc-aluminum alloy plating are twisted with a torsion angle of between 2° and 4°; the steel wire bunch is then wrapped with a polyester wrapping bandage and covered with a double-layered protective polyethylene sheath by using double-cavity co-extrusion process for one-step formation, and an outer surface of the polyethylene sheath is provided with embossments for rain-wind induced vibration resistance; the two ends of the steel wire cable are fixed by anchors using fillers, coiled, and stored. And the coils of the steel wire cables are then transported to and respectively laid on a construction field.

The present inventon provides a method for fabricating an extrusion coated steel wire cable as described in claim 1 as well as some advantageous embodiments as described in dependent claims.

To be more specific, the method comprises the following steps:

### 1) Fabricating a steel wire comprising a zinc-aluminum alloy plating

The steel wire comprising the zinc-aluminum alloy plating is adopted because the zinc-aluminum alloy plating possesses much stronger anti-corrosive property, principle of which is as follows: a) as aluminum has very active chemical property, a dense layer of alumina is formed on a surface of the steel wire after hot dip of aluminum, and therefore the surface of the steel wire is easily inactivated to form a protective layer in corrosive environment. In a corrosive medium, a zinc-enriched surface layer, functioning as a positive electrode, is firstly eroded, the aluminum content continuously increases to make the alumina content increase, thus making the plating layer possessing stronger capability of preventing external toxic substances. In the meanwhile, the addition of the aluminum also inhibits the formation of a zinc-aluminum transitional layer which has weaker anti-corrosion performance and loosen tissue, thus being helpful for improving the overall anti-corrosion performance of the plating layer. b) When the zinc-aluminum alloy plating is destructed and the steel is exposed, the plating functions as a positive electrode of an iron-zinc aluminum battery and is dissolved, and a steel substrate is therefore protected. A corrosion potential of the zinc-aluminum alloy is slightly lower than a pure zinc layer and is approximately -0.87, but the corrosion current of the zinc-aluminum alloy is only 1/5 of the hot dipped pure zinc. Under the protection of sacrificing the positive electrode, the consumption time of the zinc-aluminum alloy plating of the same amount is five folds of that of the hot dipped zinc layer. Thus, the zinc-aluminum alloy plating is able to provide much longer sacrificial protection time and possesses better endurance. The zinc-aluminum alloy plating includes two types, Zn95AI5 5 having an aluminum content of between 4.2 and 7.2 wt. %, and Zn90Al10 having the aluminum content of between 9.2 and 12.2 wt. %. A plating weight is equal to or larger than 300 g/m². A homogeneity indicator of the plating satisfies a time of copper sulfate of equal to or larger than 4 with each time lasting 60 s.

### 2) Fabricating a steel wire having a standard length

As each layer of steel wires in the stay cable exists with a certain torsion angle, it is unable to directly control the length of the steel wire cable by using the outer layers of steel wires. Only the central wire of the stay cable always remains straight without being twisted during the whole fabrication process, therefore, the central wire is utilized as the standard wire to control the overall length of the steel wire cable.

The length of the standard wire is determined by baseline measurement, and specific operation includes: applying a certain tension force to two ends of a steel wire to straighten the steel wire a performing stress correction and temperature correction using the following equation:$L = {L}_{0} \times \left[\left(1+F/EA\right)+α\left(T-20\right)\right]$ in which, L represents a length (m) of the steel wire in a stressed state, L₀ represents a designed length, *m*, of the steel wire in an unstressed state, F represents a tensioning force, *N*, E represents an elastic module, MPa, of the steel wire, and fabrication of the standard wire adopts a measured value, A represents an area of a cross section, *m*², of the steel wire, and fabrication of the standard wire adopts the measured value, α represents an expansion coefficient of the steel wire, and T represents a temperature, °*C*, of the environment.

A steel wire having a standard length is prepared. Certain markers for cutting are made at two ends of the steel wire. Thereafter, the steel wire having the standard length is utilized as a reference, and the overall length of the steel wire cable is controlled by a transfer method. By using the above measurements, the length error of the stay cable can be greatly reduced. The fabrication precision of the standard wire exceeds 1/30000, and the fabrication precision of the finished product of the steel wire cable is improved from the China's national standard of 1/5000 to 1/20000.

### 3) Twisting a bunch of steel wires

The steel wire cable is formed by multiple layers of steel wires. When supplying the steel wires, the standard wire is positioned at a center position of a cross section of the steel wire cable.

All the steel wires in the bunch are twisted to the left with a torsion angle of between 2° and 4°. The twisted steel wire bunch is wrapped by a wrapping bandage, wherein the wrapping bandage is right-handed twisted, to yield a steel wire cable as a semi-product. As lengths of the multiple layers of the steel wires are different after twisting, a length L^{/} of steel wires to be supplied for other layers surrounding the standard wire is calculated according to the following equation:${L}_{0} = {L}^{l} \times cos ⁢ α + K ,$ wherein K<0 ]in which, α represents the torsion angle ranging from 2° to 4°; K represents a fabrication allowance, *m*, which is selected according to specifications and operations; L^{/} represents the length, *m*, of other layers of the steel wires surrounding the standard wire; and L₀ represents the length, *m*, of the standard wire at the center position;

An outer dimeter of the steel wire bunch, i. e., the naked steel wire cable, after being twisted is measured. Because the cross section of the steel wire bunch is in a shape of hexagon or hexagon with missing angles, a circumscribed circle of the selected cross section of the steel wire bunch is directly the diameter of the naked steel wire cable.

The wrapping bandage is preferably a bandage made from a polyester fiber. The wrapping bandage has a width of between 40 and 60 mm and a tensile strength of equal to or high than 500 N/25 mm².

### 4) Extruding

A double-layered protective polyethylene is prepared outside the steel wire cable, in which, the double-layered protective polyethylene has a density of between 0.942 and 0.978 g/cm³, environmental stress crack resistance property of ≥ 5000 F₀/h, and a melt index of ≤ 0.45 g/10 min. Specific operation is as follows:
before extruding, a die aperture of an extruder and an extrusion velocity are preset according to an outer diameter of the steel wire cable and thicknesses of two layers of polyethylene. The double-cavity co-extrusion for one-step formation is adopted. The two layers of the polyethylene plastics simultaneously cover the steel wire cable during the requirements of anti-corrosion. According to the requirement of resistance of the rain-wind induced vibration, after the extrusion, an outer surface of the double-layered protective polyethylene is provided with helical lines or embossments. When reaching the effect of the steel wire cable in effectively inhibiting the rain-wind induced vibration, a drag coefficient is equal to or smaller than 0.8.

### 5) Accurate cutting

Original cutting positions of the steel wire cable are determined, the double-layered protective polyethylene is locally stripped, and the markers for cutting at two ends of the standard wire at the center position of the steel wire cable are found. Then, the steel wire cable is cut by using a non-liquid cutting machine and end faces of the steel wire cable are ensured perpendicular to an axis of the steel wire cable. The double-layered protective polyethylene is stripped according to a preset length to expose the steel wires, during which, the plating of the steel wires is prevented from being destructed.

### 6) Casting anchor

The anchor is a main connecting structure to transmit a tension of the steel wire cable to a tower and a girder. The steel wire cable adopts anchor structures including nut-screwing type anchor, anchor plate gap adjusting type anchor, or a fork-ear pin joint type anchor at two ends. The anchor is performed with hot galvanizing or paints coating for corrosion resistance. A thickness of the hot galvanizing is equal to or larger than 90 µm, and a thickness of the paints coating is determined according to specifications and design requirements of a steel structure. The types of the structures of the anchor is as follows:

### a) Nut-screwing type anchor

The nut screwing type anchor comprises: an anchor cup, a screw nut, an anchor plate, and a sealing assembly of a connecting cylinder. Such steel wire cable utilizes the end face of the nut to support the pressure and to transmit the load. The nut and the anchor cup are in rotary joint via a trapezoidal thread having high strength to realize the continuous adjustment of the length of the steel wire cable. The anchor cup is provided with tensional inner threads. In installation of the steel wire cable on the construction site, an installation force is applied on the steel wire cable by drawing the anchor. The anchor plate primarily functions in dispersing the steel wires, steel wire holes are distributed on the anchor plate, and the steel wires pass through corresponding steel wire holes and are headed. An external cone boss can be tightly attached to an internal conical cavity.

### b) End face-supporting type anchor

The end face-supporting type anchor comprises: an anchor cup, an anchor plate, and a sealing assembly of a connecting cylinder. End faces of such steel wire cable are directly supported on anchor plate, and different gap adjusting plates are utilized to regulate the length of the steel wire cable. The gas adjusting plates have different thicknesses to satisfy the requirement of the construction site. The anchor cup is provided with tensional inner threads. In installation of the steel wire cable on the construction site, an installation force is applied on the steel wire cable by drawing the anchor. Such kind of anchor does not necessitate nuts, and the anchor cup is not provided with external threads. The anchor plate functions in dispersing the steel wires, the steel wire holes are distributed on the anchor plate, and the steel wires pass through corresponding steel wire holes and are headed. An external cone boss can be tightly attached to an internal conical cavity.

### c) Fork-ear pin joint type anchor at one end and nut-screwing type anchor at the other end

The fork-ear pin joint type anchor comprises: a fork ear, a pin shaft, an anchor cup, a nut, and a sealing assembly of a connecting cylinder. One end of such steel wire cable is connected to the steel structure of the tower or the girder via the fork ear and the pin shaft, and the other end of the steel wire cable adopts an end face of a nut to bear pressure and to transmit the load, thus realizing the continuous adjustment of the length of the steel wire cable. the anchor cup is provided with tensional inner threads. In installation of the steel wire cable on the construction site, an installation force is applied on the steel wire cable by drawing the anchor. The anchor plate functions in dispersing the steel wires, the steel wire holes are distributed on the anchor plate, and the steel wires pass through corresponding steel wire holes and are headed. An external cone boss can be tightly attached to an internal conical cavity.

The sealing assembly of the connecting cylinder in the above three structures all adopts the new type of cable end sealing technology, in which, an outer part of the connecting cylinder is firstly sealed by a sealing cover, and an inner wall of the connecting cylinder in the vicinity of a port is sealed again by an elastic sealing ring and a sealing press ring. The two sealing measurements finally realizes the sealing of the two ends of the steel wire cable, that is, the sealing between the anchors and the interfaces of the polyethylene steel wire cable. The sealing assembly has stronger strength, thus being difficult to be destructed, much longer service life, and much endurable sealing structure.

The sealing structure at the ends of the steel wire cable is a reliable mechanical sealing structure, configured to prevent the corrosion resulting from the water penetration into the PE cable. In the meanwhile, the sealing structure, as a substitute of a heat shrink sleeve, is utilized for sealing, thus overcoming the problem of damage of the heat shrink sleeve.

The technical solution to solve the above described technical problem is as follows: an endurable sealing structure at an end of the steel wire cable. The sealing structure fits together with the connecting cylinder of the anchor and comprises: the elastic sealing ring, a sealing press ring, and a sealing cover. The sealing press ring is disposed in the port of the connecting cylinder and an outer end of the sealing press ring is exposed outside the connecting cylinder. A press surface is formed on the inner wall of the connecting cylinder relative to the inner end face of the sealing press ring. The elastic sealing ring is disposed between the inner end face of the sealing press ring and the press surface. Under the press of the press surface, the elastic sealing ring is deformed and attached to the outer wall of the steel wire cable. The sealing cover is disposed on a front end of the connecting cylinder and possesses a Harvard structure. A front part of the sealing cover contacts and fits with the outer wall of the steel wire cable and a corresponding contact surface is provided with a sealing ring. A rear part of the sealing cover contacts and fits with the sealing press ring or the connecting cylinder and a corresponding contact surface is provided with a sealing strip.

The casting of the anchor is carried out by chill casting of heading anchor or by hot casting of anchor, operations of which are as follows:

### A. Chill casting of heading anchor

a. Ends of the steel wires are fixed in anchor cups on a casting platform, oil stains and rusts are removed from portions of the steel wires inside the anchor cups, and inner walls of the anchor cups are synchronously washed.
b. The ends of the steel wires are uniformly dispersed corresponding to holes of anchor plates, and each steel wire is headed by using a heading machine. Heading dimensions are as follows: heading diameter ≥1.4 D, heading height ≥1.0 D, and D represents a diameter of the steel wires.
c. A chilled filler comprising steel balls, a stone dust, an epoxy resin, a curing agent, di-n-butyl, and a diluent is provided and uniformly mixed. A mixture of the chilled filler is poured into the anchor cups while vibrating by using a vibration pump to fully fill gaps among the anchor cup and steel wires with the mixture of the chilled filler.
d. A compression strength of the casting body of the chilled filler is ≥147 MPa.

### B. Hot casting of anchor

The hot casting anchor adopts a zinc alloy for casting, and a zinc-copper alloy and a zinc-copper-aluminum alloy are the common two alloys.

The zinc-copper alloy comprises 98 ± 0.2 wt. % of zinc and 2 ± 0.2 wt. % of copper, and the zinc-copper-aluminum alloy comprises 4 - 7 wt. % of aluminum, 1 - 2 wt. % of copper, and 91 - 95 wt. % of zinc. The casting is performed as follows:
a. Ends of the steel wires are perpendicularly fixed in anchor cups on the casting platform, steel wires comprising a zinc-aluminum alloy plating are dispersed inside the anchor cups in the form of concentric circles. Oil stains and rusts are then removed from surfaces of the steel wires, and the inner walls of the anchor cups are simultaneously washed.
b. The center of the steel wire cable is kept coincide with centers of the anchor cups, and steel wires are prevented from contacting the anchor cups.
c. Bottom openings of the anchor cups are sealed to prevent the alloy from leaking via the bottom openings. The anchor cups are preheated.
d. The zinc-copper alloy or the zinc-copper-aluminum alloy is poured into the anchor cups for one-step casting while avoiding any vibration or disruption.

### 7) Performing tension detection or top pressure detection

The tension detection or the top pressure detection are important means to detect the quality of the steel wire cable. According to fillers for the casting of the anchor, the tension detection is performed on the steel wire cable with chilled-casted anchor or the top pressure detection is performed on the steel wire cable with hot-casted anchor before leaving a plant, which is specifically as follows:

For the steel wire cable with the chilled-casted anchor, the steel wire cable is stretched by an overstretching force which is set to be between 1.1 and 1.5 folds of a designed tension of the steel wire cable and satisfies that a retraction value of a casting body inside the anchor cup after stretching is equal to or less than 6 mm.

The overstretching force is then unloaded to be 20% of the original overstretching force or to be the designed tension of the steel wire cable after the stretching. A length of the steel wire cable is measured at a stable temperature in the dark, and a stressless length of the steel wire cable is calculated at a reference temperature according to the following equation:${L}_{CO} = \frac{{L}_{CP}}{1 + \frac{{P}_{20}}{EA} + α \left(t-{t}_{0}\right)}$ in which, L_{C0} represents the stressless length, *m*, of the steel wire cable at the reference temperature; L_{CP} represents a length, *m*, of the steel wire cable loaded with a tension force of P₂₀; P₂₀ represents 20% of the overstretching force, *N*; A represents a nominal area, *mm²,* of the steel wire bunch of the steel wire cable; E represents an elastic modulus, *MPa*; α represents a coefficient of linear expansion of a stay cable which is equal to 0.000012/°C; t represents the stable temperature, °*C*, when measuring a length of the stay cable; and t₀ represents a designed reference temperature, °*C*, of the stay cable.

For the steel wire cable with hot-casted anchor, Atop pressure is applied to the steel wire cable. The top pressure is 1.25 folds of the designed tension of the steel wire cable and satisfies that a retraction value of the casting body inside the anchor cup after the top pressure detection is equal to or less than 6 mm.

### 8) Coiling

The steel wire cable is coiled by a coil frame. Before the coiling, an outer surface of the steel wire cable is packed, and layers of the steel wire cables are successively coiled by using the coil frame. An inner diameter of a resulting coil is equal to or larger than 20 folds of an outer diameter of the steel wire cable and is equal to or larger than 1.6 m.

### 9) Storing

Finished product of the steel wire cable adopts indoor storage or outdoor storage. When the indoor storage is adopted, an oilcloth is used to cover the steel wire cable. A storage site is equipped with ventilation and fire-proof facilities to ensure the quality and the safety of the stored steel wire cables.

Compared with the prior art, the method for fabricating the steel wire cable comprising the extruded polyethylene and the zinc-aluminum alloy plating has the following advantages: the steel wires are arranged according to the arrangement rule at the cross section of the steel wire cable. The length of the overall cable is controlled by the length of the central standard wire. The bunch of the steel wires comprising the zinc-aluminum alloy plating are twisted with the torsion angle of between 2° and 4°. The steel wire bunch is then wrapped with the polyester wrapping bandage and covered with the double-layered protective polyethylene sheath by using double-cavity co-extrusion process for one-step formation, and the outer surface of the polyethylene sheath is provided with embossments for rain-wind induced vibration resistance. The two ends of the steel wire cable are fixed by anchors using fillers, coiled, and stored. And the coils of the steel wire cables are then transported to and respectively laid on the construction field. The fabrication of the steel wire cable of the invention is not restricted by the construction site, and hardly affected by the climate factors. And the management of the industrialized production is easily controllable. All these satisfy the use requirements of long length, high accuracy, and endurance of the stay cable for the large-span bridge used in the marine environment.
FIG. **1** is a structure diagram illustrating two nut-screwing type anchors at two ends of a steel wire cable;
FIG. **2** is a structure diagram illustrating two anchor plate gap adjusting type anchors at two ends of a steel wire cable;
FIG. **3** is a structure diagram illustrating a fork-ear pin joint type anchor at one end of a steel wire cable and a nut-screwing type anchor at the other end of the steel wire cable; and
FIG. **4** is a side view of FIG. **3****.**

In the drawings, the following numbers are utilized: **1.** Anchor plate; **2.** Anchor cup; **3.** Sealing assembly of a connecting cylinder; **4.** Steel wire cable; **5.** Sealing structure at an end of a steel wire cable; **6.** Nut; **7.** Gap adjusting plate; **8.** Pin shaft; and **9.** Fork ear.

For further illustrating the invention, experiments detailing a method for fabricating a steel wire cable comprising an extruded polyethylene and a zinc-aluminum alloy plating are described below. It should be noted that the following examples are intended to describe and not to limit the invention.

In the method of the invention, steel wires comprising a zinc-aluminum alloy plating are twisted together to form a naked steel wire cable, an outer layer of the naked steel wire cable is covered by a double-layered protective polyethylene by extrusion. Two ends of a resulting steel wire cable are then anchored by casting, coiled, transported to the construction site and laid respectively.

### 1) fabricating a steel wire comprising a zinc-aluminum alloy plating

The steel wire comprising the zinc-aluminum alloy plating is adopted because the zinc-aluminum alloy plating possesses much stronger anti-corrosive property. The zinc-aluminum alloy plating includes two types, Zn95AI5 5 having an aluminum content of between 4.2 and 7.2 wt. %, and Zn90Al10 having the aluminum content of between 9.2 and 12.2 wt. %. A plating weight is equal to or larger than 300 g/m².

### 2) fabricating a steel wire having a standard length

As each layer of steel wires in the stay cable exists with a certain torsion angle, it is unable to directly control the length of the steel wire cable by using the outer layers of steel wires. Only the central wire of the stay cable always remains straight without being twisted during the whole fabrication process, therefore, the central wire is utilized as the standard wire to control the overall length of the steel wire cable.

The length of the standard wire is determined by baseline measurement, and specific operation includes: applying a certain tension force to two ends of a steel wire to straighten the steel wire a performing stress correction and temperature correction using the following equation:$L = {L}_{0} \times \left[\left(1+F/EA\right)+α\left(T-20\right)\right]$ in which, L represents a length (m) of the steel wire in a stressed state, L₀ represents a designed length, *m*, of the steel wire in an unstressed state, F represents a tensioning force, *N*, E represents an elastic module, *MPa*, of the steel wire, and fabrication of the standard wire adopts a measured value, A represents an area of a cross section, *m²*, of the steel wire, and fabrication of the standard wire adopts the measured value, α represents an expansion coefficient of the steel wire, and T represents a temperature, °C, of the environment.

A steel wire having a standard length is prepared. Certain markers for cutting are made at two ends of the steel wire. Thereafter, the steel wire having the standard length is utilized as a reference, and the overall length of the steel wire cable is controlled by a transfer method.

### 3) twisting a steel wire bunch

The steel wire cable is formed by multiple layers of steel wires. When relaxing the steel wires, the standard wire is positioned at a center position of a cross section of the steel wire cable.

A steel wire bunch is twisted to the left with a torsion angle of between 2° and 4°. The twisted steel wire bunch is wrapped by a wrapping bandage, wherein the wrapping bandage is right-handed twisted, to yield a steel wire cable as a semi-product. As lengths of the multiple layers of the steel wires exist with differences, a length L^{/} of steel wires to be supplied for other layers of steel wires surrounding the standard wire considering the length of the standard wire is calculated according to the following equation:${L}_{0} = {L}^{l} \times cos ⁢ α + K ,$ wherein K<0 in which, α represents the torsion angle ranging from 2° to 4°; K represents a fabrication allowance, m, which is selected according to specifications and operations; L^{/} represents the length, m, of other layers of the steel wires surrounding the standard wire; and L₀ represents the length, m, of the standard wire at the center position;

An outer diameter of the steel wire bunch, i. e., the naked steel wire cable, after being twisted is measured. Because the cross section of the steel wire bunch is in a shape of hexagon, a circumscribed circle of the selected cross section of the steel wire bunch is directly the diameter of the naked steel wire cable.

### 4) extruding

A double-layered protective polyethylene is prepared outside the steel wire cable. Before extruding, a die aperture of an extruder and an extrusion velocity are preset according to an outer diameter of the steel wire cable and thicknesses of two layers of polyethylene. The double-cavity co-extrusion for one-step formation is adopted. The two layers of the polyethylene plastics simultaneously cover the steel wire cable during the requirements of anti-corrosion.

According to the requirement of resistance of the rain-wind induced vibration, after the extrusion, an outer surface of the double-layered protective polyethylene is provided with helical lines or embossments. When reaching the effect of the steel wire cable in effectively inhibiting the rain-wind induced vibration, a drag coefficient is equal to or smaller than 0.8.

### 5) accurate cutting

Original cutting positions of the steel wire cable are determined, the double-layered protective polyethylene is locally stripped, and the markers for cutting at two ends of the standard wire at the center position of the steel wire cable are found. Then, the steel wire cable is cut by using a non-liquid cutting machine and end faces of the steel wire cable are ensured perpendicular to an axis of the steel wire cable. The double-layered protective polyethylene is stripped according to a preset length to expose the steel wires, during which, the plating of the steel wires is prevented from being destructed.

### 6) casting anchor

The anchor is a main connecting structure to transmit a tension of the steel wire cable to a tower and a girder. Anchor structures of the steel wire cable are as follows: two nut-screwing type anchors disposed at two ends of the steel wire cable, as shown in FIG. **1****,** two anchor plate gap adjusting type anchors at two ends of the steel wire cable, as shown in FIG. **2****,** and a fork-ear pin joint type anchor at one end of the steel wire cable and a nut-screwing type anchor at the other end of the steel wire cable, as shown in FIGS. **3-4****.**

### a) Nut-screwing type anchor

The nut screwing type anchor comprises: an anchor cup, a screw nut, an anchor plate, and a sealing assembly of a connecting cylinder. Such steel wire cable utilizes the end face of the nut to support the pressure and to transmit the load. The nut and the anchor cup are in rotary joint via a trapezoidal thread having high strength to realize the continuous adjustment of the length of the steel wire cable. The anchor cup is provided with tensional inner threads. In installation of the steel wire cable on the construction site, an installation force is applied on the steel wire cable by drawing the anchor. The anchor plate primarily functions in dispersing the steel wires, steel wire holes are distributed on the anchor plate, and the steel wires pass through corresponding steel wire holes and are headed. An external cone boss can be tightly attached to an internal conical cavity.

### b) End face-supporting type anchor

The end face-supporting type anchor comprises: an anchor cup, an anchor plate, and a sealing assembly of a connecting cylinder. End faces of such steel wire cable are directly supported on anchor plate, and different gap adjusting plates are utilized to regulate the length of the steel wire cable. The gas adjusting plates have different thicknesses to satisfy the requirement of the construction site. The anchor cup is provided with tensional inner threads. In installation of the steel wire cable on the construction site, an installation force is applied on the steel wire cable by drawing the anchor. Such kind of anchor does not necessitate nuts, and the anchor cup is not provided with external threads. The anchor plate functions in dispersing the steel wires, the steel wire holes are distributed on the anchor plate, and the steel wires pass through corresponding steel wire holes and are headed. An external cone boss can be tightly attached to an internal conical cavity.

### c) Fork-ear pin joint type anchor at one end and nut-screwing type anchor at the other end

The fork-ear pin joint type anchor comprises: a fork ear, a pin shaft, an anchor cup, a nut, and a sealing assembly of a connecting cylinder. One end of such steel wire cable is connected to the steel structure of the tower or the girder via the fork ear and the pin shaft, and the other end of the steel wire cable adopts an end face of a nut to bear pressure and to transmit the load, thus realizing the continuous adjustment of the length of the steel wire cable. the anchor cup is provided with tensional inner threads. In installation of the steel wire cable on the construction site, an installation force is applied on the steel wire cable by drawing the anchor. The anchor plate functions in dispersing the steel wires, the steel wire holes are distributed on the anchor plate, and the steel wires pass through corresponding steel wire holes and are headed. An external cone boss can be tightly attached to an internal conical cavity.

The sealing assembly of the connecting cylinder in the above three structures all adopts the new type of cable end sealing technology, in which, an outer part of the connecting cylinder is firstly sealed by a sealing cover, and an inner wall of the connecting cylinder in the vicinity of a port is sealed again by an elastic sealing ring and a sealing press ring. The two sealing measurements finally realizes the sealing of the two ends of the steel wire cable, that is, the sealing between the anchors and the interfaces of the polyethylene steel wire cable. The sealing assembly has stronger strength, thus being difficult to be destructed, much longer service life, and much endurable sealing structure.

The sealing structure at the ends of the steel wire cable is a reliable mechanical sealing structure, configured to prevent the corrosion resulting from the water penetration into the PE cable. In the meanwhile, the sealing structure, as a substitute of a heat shrink sleeve, is utilized for sealing, thus overcoming the problem of damage of the heat shrink sleeve.

The technical solution to solve the above described technical problem is as follows: an endurable sealing structure at an end of the steel wire cable. The sealing structure fits together with the connecting cylinder of the anchor and comprises: the elastic sealing ring, a sealing press ring, and a sealing cover. The sealing press ring is disposed in the port of the connecting cylinder and an outer end of the sealing press ring is exposed outside the connecting cylinder. A press surface is formed on the inner wall of the connecting cylinder relative to the inner end face of the sealing press ring. The elastic sealing ring is disposed between the inner end face of the sealing press ring and the press surface. Under the press of the press surface, the elastic sealing ring is deformed and attached to the outer wall of the steel wire cable. The sealing cover is disposed on a front end of the connecting cylinder and possesses a Harvard structure. A front part of the sealing cover contacts and fits with the outer wall of the steel wire cable and a corresponding contact surface is provided with a sealing ring. A rear part of the sealing cover contacts and fits with the sealing press ring or the connecting cylinder and a corresponding contact surface is provided with a sealing strip.

The anchor is performed with hot galvanizing or paints coating for corrosion resistance. A thickness of the hot galvanizing is equal to or larger than 90 µm, and a thickness of the paints coating is determined according to specifications and design requirements of a steel structure.

The casting of the anchor is carried out by chill casting of heading anchor or by hot casting of anchor, operations of which are as follows:

### A. Chill casting of heading anchor

a. Ends of the steel wires are fixed in anchor cups on a casting platform, oil stains and rusts are removed from portions of the steel wires inside the anchor cups, and inner walls of the anchor cups are synchronously washed.
b. The ends of the steel wires are uniformly dispersed corresponding to holes of anchor plates, and each steel wire is headed by using a heading machine. Heading dimensions are as follows: heading diameter ≥1.4 D, heading height ≥1.0 D, and D represents a diameter of the steel wires.
c. A chilled filler comprising steel balls, a stone dust, an epoxy resin, a curing agent, di-n-butyl, and a diluent is provided and uniformly mixed. A mixture of the chilled filler is poured into the anchor cups while vibrating by using a vibration pump to fully fill gaps among the anchor cup and steel wires with the mixture of the chilled filler.

### B. Hot casting of anchor

The hot casting anchor adopts a zinc alloy for casting, and a zinc-copper alloy and a zinc-copper-aluminum alloy are the common two alloys.

The zinc-copper alloy comprises 98 ± 0.2 wt. % of zinc and 2 ± 0.2 wt. % of copper, and the zinc-copper-aluminum alloy comprises 4 - 7 wt. % of aluminum, 1 - 2 wt. % of copper, and 91 - 95 wt. % of zinc. The casting is performed as follows:
a. Ends of the steel wires are perpendicularly fixed in anchor cups on the casting platform, steel wires comprising a zinc-aluminum alloy plating are dispersed inside the anchor cups in the form of concentric circles. Oil stains and rusts are then removed from surfaces of the steel wires, and the inner walls of the anchor cups are simultaneously washed.
b. The center of the steel wire cable is kept coincide with centers of the anchor cups, and steel wires are prevented from contacting the anchor cups.
c. Bottom openings of the anchor cups are sealed to prevent the alloy from leaking via the bottom openings. The anchor cups are preheated.
d. The zinc-copper alloy or the zinc-copper-aluminum alloy is poured into the anchor cups for one-step casting while avoiding any vibration or disruption.

### 7) Performing tension detection or top pressure detection

The tension detection or the top pressure detection are important means to detect the quality of the steel wire cable. According to fillers for the casting of the anchor, the tension detection is performed on the steel wire cable with chilled-casted anchor or the top pressure detection is performed on the steel wire cable with hot-casted anchor before leaving a plant, which is specifically as follows:

For the steel wire cable with the chilled-casted anchor, the steel wire cable is stretched by an overstretching force which is set to be between 1.1 and 1.5 folds of a designed tension of the steel wire cable and satisfies that a retraction value of a casting body inside the anchor cup after stretching is equal to or less than 6 mm.

The overstretching force is then unloaded to be 20% of the original overstretching force or to be the designed tension of the steel wire cable after the stretching. A length of the steel wire cable is measured at a stable temperature in the dark, and a stressless length of the steel wire cable is calculated at a reference temperature according to the following equation:${L}_{CO} = \frac{{L}_{CP}}{1 + \frac{{P}_{20}}{EA} + α \left(t-{t}_{0}\right)}$ in which, L_{C0} represents the stressless length, *m*, of the steel wire cable at the reference temperature; L_{CP} represents a length, *m*, of the steel wire cable loaded with a tension force of P₂₀; P₂₀ represents 20% of the overstretching force, *N*; A represents a nominal area, *mm²,* of the steel wire bunch of the steel wire cable; E represents an elastic modulus, *MPa;* α represents a coefficient of linear expansion of a stay cable which is equal to 0.000012/°C; t represents the stable temperature, °*C*, when measuring a length of the stay cable; and t₀ represents a designed reference temperature, °*C*, of the stay cable.

An error of the stressless length of the steel wire cable at the reference temperature satisfies the following requirements:
when L_{C0} ≤ 100 m, the error is less than or equal to 10 mm; and
when L_{C0} > 100 m, the error is less than or equal to L_{C0}/20000 + 5 mm.

For the steel wire cable with hot-casted anchor, a top pressure is applied to the steel wire cable. The top pressure is 1.25 folds of the designed tension of the steel wire cable and satisfies that a retraction value of the casting body inside the anchor cup after the top pressure detection is equal to or less than 6 mm.

### 8) Coiling

The steel wire cable is coiled by a coil frame. Before the coiling, an outer surface of the steel wire cable is packed, and layers of the steel wire cables are successively coiled by using the coil frame. An inner diameter of a resulting coil is equal to or larger than 20 folds of an outer diameter of the steel wire cable and is equal to or larger than 1.6 m.

### 9) Storing

Finished product of the steel wire cable adopts indoor storage or outdoor storage. When the indoor storage is adopted, an oilcloth is used to cover the steel wire cable. A storage site is equipped with ventilation and fire-proof facilities to
ensure the quality and the safety of the stored steel wire cables.

## Claims

1. A method for fabricating an extrusion coated steel wire cable, the method comprising the steps of:
1) fabricating a steel wire comprising a zinc-aluminum alloy plating, including
preparing a zinc-aluminum alloy plating on a surface of the steel wire, in which, the zinc-aluminum alloy adopts a Zn95Al5 having an aluminum content of between 4.2 and 7.2 wt. % or a Zn90Al10 having the aluminum content of between 9.2 and 12.2 wt. %, and a weight of the zinc-aluminum alloy plating is equal to or larger than 300 g/m²;
2) fabricating a steel wire having a standard length from said wire obtained by step 1), including
making a central wire as a standard wire and determining a length of the standard wire by baseline measurement, applying a certain tension force to two ends of a steel wire to straighten the steel wire and performing stress correction and temperature correction to prepare a steel wire having a standard length; making certain markers for cutting at two ends of the steel wire; making the steel wire having the standard length as a reference, and controlling an overall length of the steel wire cable by a transfer method;
3) twisting a bunch of steel wires into a steel wire cable, including
supplying steel wires obtained by step 1),
positioning the standard wire at a center position of a cross section of the steel wire cable to be formed by a plurality of layers of the steel wires;
twisting all the steel wires in the bunch to the left with a torsion angle α of between 2° and 4° thereby obtaining a naked steel wire cable;
and wrapping the naked steel wire cable by a wrapping bandage, wherein the wrapping bandage is right-handed twisted, to yield a steel wire cable as a semi-product;
wherein the length L^{/} of the steel wires to be supplied for said plurality of layers surrounding the standard wire is calculated by considering the length of the standard wire and the torsion angle α according to the following equation: ${L}_{0} = {L}^{l} \times cos ⁢ α + K ,$ wherein K<0
in which,
α represents the torsion angle ;
K is in meters (*m*) and is selected according to specifications and operations;
L^{/} represents the length in meters (*m*) of the steel wires to be supplied for the layers surrounding the standard wire;
and L₀ represents the length in meters (*m*) of the standard wire at the center position;
4) extruding, including
preparing a double-layered protective polyethylene outside the steel wire cable of step 3), in which the double-layered protective polyethylene has a density of between 0.942 and 0.978 g/cm³, environmental stress crack resistance property of ≥ 5000 F₀/h, and a melt index of ≤ 0.45 g/10 min; before extruding, presetting a die aperture of an extruder and an extrusion velocity according to an outer diameter of the steel wire cable and thicknesses of two layers of polyethylene; in which, the die aperture of the extruder is provided with two layers of discharge channel, and the two layers of polyethylene simultaneously cover the steel wire cable during the extrusion;
wherein a magnetic field is arranged above the steel wire cable to make the steel wire cable in a suspension state; after the extrusion process, the double-layered protective polyethylene and the naked steel wire cable are concentrically arranged;
5) cutting, including
determining original cutting positions of the extrusion coated steel wire cable, by locally stripping the double-layered protective polyethylene, finding the markers for cutting at two ends of the standard wire at the center position of the extrusion coated steel wire cable;
cutting the extrusion coated steel wire cable by using a non-liquid cutting machine and ensuring end faces of the extrusion coated steel wire cable perpendicular to an axis of the extrusion coated steel wire cable;
stripping the double-layered protective polyethylene according to a preset length to expose the steel wires;
6) casting an anchor to the extrusion coated steel wire cable of step 5), including
providing an anchor functioning as a main connecting structure to transmit a tension of the extrusion coated steel wire cable to a tower or a girder; including
performing hot galvanizing or paints coating on the anchor for corrosion resistance, in which, a thickness of the hot galvanizing is equal to or larger than 90 µm, and a thickness of the paints coating is determined according to specifications and design requirements of - steel structure;
casting the anchor by chill casting of a heading anchor or by hot casting of an anchor, operations of which are as follows:
A. chill casting of a heading anchor, including
a. fixing ends of the steel wires in anchor cups on a casting platform, removing oil stains and rusts from portions of the steel wires inside the anchor cups, and synchronously washing inner walls of the anchor cups;
b. uniformly dispersing the ends of the steel wires corresponding to holes of anchor plates, and heading each steel wire by using a heading machine, in which, heading dimensions are as follows: heading diameter ≥1.4 D, heading height ≥1.0 D, and D represents a diameter of the steel wires;
c. providing and uniformly mixing a chilled filler comprising steel balls, a stone dust, an epoxy resin, a curing agent, di-n-butyl, and a diluent; pouring a mixture of the chilled filler into the anchor cups while vibrating by using a vibration pump to fully fill gaps among the anchor cup and steel wires with the mixture of the chilled filler; or
B. hot casting of anchor, including
providing a zinc-copper alloy comprising 98 ± 0.2 wt. % of zinc and 2 ± 0.2 wt. % of copper, or a zinc-copper-aluminum alloy comprising 4 - 7 wt. % of aluminum, 1 - 2 wt. % of copper, and 91 - 95 wt. % of zinc; and performing casting as follows:
a. perpendicularly fixing ends of the steel wires in anchor cups on the casting platform, dispersing steel wires comprising a zinc-aluminum alloy plating inside the anchor cups in the form of concentric circles, removing oil stains and rusts from surfaces of the steel wires, and simultaneously washing the inner walls of the anchor cups;
b. keeping the center of the steel wire cable coincide with centers of the anchor cups and preventing steel wires from contacting the anchor cups;
c. sealing bottom openings of the anchor cups to prevent the alloy from leaking via the bottom openings; and preheating the anchor cups;
d. pouring the zinc-copper alloy or the zinc-copper-aluminum alloy into the anchor cups for one-step casting while avoiding any vibration or disruption;
7) performing tension detection or top pressure detection, including
according to fillers for the casting of the anchor, performing tension detection on the steel wire cable with chilled-casted anchor or performing top pressure detection on the steel wire cable with hot-casted anchor before leaving a plant, which is specifically as follows:
for the steel wire cable with the chilled-casted anchor, stretching the steel wire cable by an overstretching force which is set to be between 1.1 and 1.5 folds of a designed tension of the steel wire cable and satisfies that a retraction value of a casting body inside the anchor cup after stretching is equal to or less than 6 mm;
unloading the overstretching force to be 20% of the original overstretching force or to be the designed tension of the steel wire cable after the stretching; measuring a length of the steel wire cable at a constant temperature in the dark, and calculating a stressless length of the steel wire cable at a reference temperature according to the following equation: ${L}_{CO} = \frac{{L}_{CP}}{1 + \frac{{P}_{20}}{EA} + α \left(t-{t}_{0}\right)}$ in which,
L_{C0} represents the stressless length in meters (m) of the steel wire cable at the reference temperature;
L_{CP} represents a length in meters (m) of the steel wire cable loaded with a tension force of P₂₀;
P₂₀ represents 20% of the overstretching force in *N*;
A represents a nominal area in mm² of the naked steel wire cable;
E represents an elastic modulus in MPa;
α represents a coefficient of linear expansion of a steel wire cable which is equal to 0.000012/°C;
t represents a stable temperature in °C when measuring a length of the steel wire cable;
and t₀ represents a designed reference temperature in °C of the steel wire cable;
for the steel wire cable with the hot-cast anchor, applying, to the steel wire cable, a top pressure which is 1.25 folds of the designed tension of the steel wire cable and satisfies that a retraction value of the casting body inside the anchor cup after the top pressure detection is equal to or less than 6 mm; and
8) coiling the finished extrusion coated steel wire cable of step 7), including
coiling layers of the finished extrusion coated steel wire cable successively by using a coil frame, in which, an inner diameter of a resulting coil is equal to or larger than 20 folds of an outer diameter of the steel wire cable and is equal to or larger than 1.6 m.

2. The method of claim 1, **characterized in that** when determining the length of the standard wire in step 2), stress correction and temperature correction are then carried out according to the following equation: $L = {L}_{0} \times \left[\left(1+F/EA\right)+α\left(T-20\right)\right]$ in which,
L represents a length in m of the steel wire in a stressed state,
L₀ represents a designed length in m of the steel wire in an unstressed state,
F represents a tensioning force in *N,*
E represents an elastic module in MPa of the steel wire, wherein fabrication of the standard wire adopts a measured value,
A represents an area of a cross section in m² of the steel wire, wherein fabrication of the standard wire adopts a measured value,
α represents an expansion coefficient of the steel wire,
and T represents a temperature of the environment.

3. The method of claim 1, **characterized in that** an outer surface of the double-layered protective polyethylene is provided with helical lines or embossments, and a drag coefficient is equal to or smaller than 0.8.

4. The method of claim 1, **characterized in that** structures of the anchors in step 6) adopt a nut-screwing type anchor, an anchor plate gap adjusting type anchor, or a fork-ear pin joint type anchor at two ends of the steel wire cable.

5. The method of claim 1, **characterized in that** in step 7), an error of the stressless length of the steel wire cable at the reference temperature satisfies the following requirements:
when L_{C0} ≤ 100 m, the error is less than or equal to 10 mm; and
when L_{C0} > 100 m, the error is less than or equal to L_{C0}/20000 + 5 mm.

6. The method of claim 1, **characterized in that** the wrapping bandage is a bandage made from polyester fibers; the wrapping bandage has a width of between 40 and 60 mm and a tensile strength of equal to or higher than 500 N/25 mm².

## Patentansprüche

1. Verfahren zur Herstellung eines umspritzten Stahldrahtseils, wobei das Verfahren die folgenden Schritte aufweist:
1) Herstellung eines Stahldrahts mit einer Zink-Aluminium-Legierungsbeschichtung, umfassend
das Aufbringen einer Zink-Aluminium-Legierungsbeschichtung auf eine Oberfläche des Stahldrahts, bei welcher Beschichtung die Zink-AluminiumLegierung eine Zn95Al5-Legierung mit einem Aluminiumgehalt von zwischen 4,2 und 7,2 Gew.-% oder eine Zn90Al10-Legierung mit einem Aluminiumgehalt von zwischen 9,2 und 12,2 Gew.-% aufweist und ein Gewicht der Zink-Aluminium-Legierungsbeschichtung gleich oder größer 300 g/m² ist;
2) Herstellung eines Stahldrahts mit einer Standardlänge aus dem in Schritt 1) erhaltenen Draht, umfassend
Nehmen eines zentralen Drahts als Standarddraht und Bestimmung einer Länge des Standarddrahts durch Basismessung, Anlegen einer bestimmten Spannkraft an beide Enden eines Stahldrahts, um den Stahldraht gerade zu ziehen, und Durchführung einer Spannungskorrektur und Temperaturkorrektur zur Herstellung eines Stahldrahts mit einer Standardlänge; Setzen bestimmter Markierungen zum Schneiden an beiden Enden des Stahldrahts; Nehmen des Stahldrahts mit der Standardlänge als Bezugsdraht und Steuern einer Gesamtlänge des Stahldrahtseils durch ein Übertragungsverfahren;
3) Verdrillen eines Bündels aus Stahldrähten zu einem Stahldrahtseil, umfassend
das Liefern von durch Schritt 1) erhaltenen Stahldrähten,
die Positionierung des Standarddrahts an einer mittleren Position eines Querschnitts des Stahldrahtseils, das durch eine Vielzahl von Schichten an Stahldrähten ausgebildet werden soll;
das Verdrillen aller Stahldrähte in dem Bündel nach links mit einem Torsionswinkel α von zwischen 2° und 4°, wodurch ein nacktes Stahldrahtseil erhalten wird;
und Umwickeln des nackten Stahldrahtseils mit einer Umhüllungsbandage, wobei die Umhüllungsbandage rechtsherum gedreht wird, um ein Stahldrahtseil als ein halbfertiges Produkt zu erhalten;
wobei die Länge L' der Stahldrähte, die für die Vielzahl von den Standarddraht umgebenden Schichten zu liefern sind, berechnet wird unter Berücksichtigung der Länge des Standarddrahts und des Torsionswinkels α gemäß der folgenden Gleichung : ${L}_{0} = L ′ \times cosa + K ,$ wobei K < 0 wobei
α den Torsionswinkel darstellt;
K in Metern (*m*) angegeben ist und gemäß Spezifikationen und Operationen ausgewählt wird;
L' die Länge in Metern (*m*) der Stahldrähte darstellt, die für die den Standarddraht umgebenden Schichten zu liefern sind;
und L₀ die Länge in Metern (*m*) des Standarddrahts in der mittleren Position darstellt;
4) Extrudieren, umfassend
die Herstellung eines doppellagigen Schutzfilms aus Polyethylen außerhalb des Stahldrahtseils aus Schritt 3), wobei der doppellagige Schutzfilm aus Polyethylen eine Dichte von zwischen 0,942 und 0,978 g/cm³, eine Spannungsrissbeständigkeit von ≥ 5000 F₀/h und einen Schmelzindex von < 0,45 g/10 min aufweist; vor dem Extrudieren eine Voreinstellung einer Düsenöffnung eines Extruders und einer Extrudiergeschwindigkeit gemäß einem Außendurchmesser des Stahldrahtseils und der Dicke zweier Schichten aus Polyethylen; wobei die Düsenöffnung des Extruders mit zwei Schichten eines Entladungskanals versehen ist, und die beiden Polyethylenschichten gleichzeitig während des Extrudierens das Stahldrahtseil bedecken;
wobei ein Magnetfeld oberhalb des Stahldrahtseils angeordnet ist, um das Stahldrahtseil in einen Schwebezustand zu versetzen; wobei der doppellagige Schutzfilm aus Polyethylen und das nackte Stahldrahtseil nach dem Extrudiervorgang konzentrisch angeordnet werden;
5) Schneiden, umfassend
die Bestimmung ursprünglicher Schneidepositionen an dem umspritzten Stahldrahtseil, indem örtlich der doppellagige Schutzfilm aus Polyethylen abgezogen wird, und Finden der Markierungen zum Schneiden an beiden Enden des Standarddrahts in der mittleren Position des umspritzten Stahdrahtseils;
das Schneiden des umspritzten Stahldrahtseils unter Verwendung einer nicht flüssigen Schneidemaschine und Sicherstellen von Endflächen des umspritzten Stahldrahtseils, die senkrecht zu einer Achse des umspritzten Stahldrahtseils liegen;
das Abziehen des doppellagigen Schutzfilms aus Polyethylen gemäß einer vorbestimmten Länge, um die Stahldrähte freizulegen;
6) Gießen eines Ankers an das umspritzte Stahldrahtseil aus Schritt 5), umfassend
die Bereitstellung eines Ankers, der als Hauptverbindungsstruktur fungiert, um eine Spannung des umspritzten Stahldrahtseils auf einen Mast oder einen Träger zu übertragen; umfassend
die Durchführung einer Feuerverzinkung oder einer Lackbeschichtung an dem Anker zum Widerstand gegen Korrosion, wobei eine Dicke der Feuerverzinkung gleich oder größer 90 µm ist, und eine Dicke der Lackbeschichtung gemäß Spezifikationen und Designanforderungen der Stahlstruktur festgelegt wird;
das Gießen des Ankers mittels Kaltgießen eines Stauchankers oder mittels Heißgießens eines Ankers, wobei die Vorgänge wie nachfolgend erläutert erfolgen:
A. Kaltgießen eines Stauchankers, umfassend
a. Befestigung der Enden der Stahldrähte in Ankerschalen auf einer Gussplattform, Entfernen von Öl- und Rostflecken an Bereichen der Stahldrähte innerhalb der Ankerschalen und gleichzeitiges Waschen der Innenwände der Ankerschalen;
b. gleichmäßige Verteilung der Enden der Stahldrähte entsprechend den Löchern von Ankerplatten und Stauchen jedes Stahldrahts unter Verwendung einer Stauchmaschine, wobei die Stauchabmessungen die folgenden sind: Stauchdurchmesser: ≥ 1,4 D, Stauchhöhe ≥ 1,0 D und D stellt einen Durchmesser der Stahldrähte dar;
c. Bereitstellen und gleichmäßiges Mischen eines gekühlten Füllmaterials, welches Stahlkugeln, Steinstaub, ein Epoxidharz, einen Härter, Di-n-butyl und ein Verdünnungsmittel aufweist; Gießen einer Mischung des gekühlten Füllmaterials in die Ankerschalen unter Vibrieren durch Verwendung einer Vibrationspumpe, um Spalten zwischen den Ankertassen und Stahldrähten vollständig mit der Mischung des gekühlten Füllmaterials auszufüllen; oder
B. Heißgießen eines Ankers, umfassend
die Bereitstellung einer Zink-Kupfer-Legierung mit 98 ± 0,2 Gew,-% Zink und 2 ± 0,2 Gew.-% Kupfer, oder einer Zink-Kupfer-Legierung mit 4 - 7 Gew,-% Aluminium, 1 - 2 Gew,-% Kupfer und 91 - 95 Gew.-% Zink; und Durchführung des Gießens wie folgt:
a. senkrechte Befestigung der Enden der Stahldrähte in den Ankerschalen auf der Gussplattform, Verteilung der Stahldrähte, welche eine Zink-Aluminium-Legierungsbeschichtung aufweisen, innerhalb der Ankerschalen in Form von konzentrischen Kreisen, Entfernen von Öl- und Rostflecken von Oberflächen der Stahldrähte und gleichzeitiges Waschen der Innenwände der Ankerschalen;
b. Halten des Mittelpunkts des Stahldrahtseils in Übereinstimmung mit den Mittelpunkten der Ankerschalen und Vermeiden, dass die Stahldrähte die Ankerschalen berühren;
c. Abdichten der unteren Öffnungen der Ankerschalen, um zu verhindern, dass die Legierung durch die unteren Öffnungen herausläuft, und Vorheizen der Ankerschalen;
d. Gießen der Zink-Kuper-Legierung oder der Zink-Kupfer-AluminiumLegierung in die Ankerschalen in einem einstufigen Guss, wobei jegliche Vibration oder Unterbrechung vermieden wird;
7) Durchführung einer Spannungserfassung oder einer Spitzendruckerfassung, umfassend
gemäß den Füllstoffen für das Gießen des Ankers, Durchführung einer Spannungserfassung an dem Stahldrahtseil bei einem kalt gegossenen Anker oder Durchführung einer Spitzendruckerfassung an dem Stahldrahtseil bei einem heiß gegossenen Anker vor Verlassen der Anlage, welche Erfassungen insbesondere wie folgt ablaufen:
bei dem Stahldrahtseil mit dem kalt gegossenen Anker wird das Stahldrahtseil mit einer Überdehnungskraft gespannt, die so eingestellt ist, dass sie zwischen dem 1,1-fachen und 1,5-fachen einer für das Stahldrahtseil konzipierten Spannung liegt und erfüllt, dass ein Rückzugswert eines Gusskörpers innerhalb der Ankerschale nach dem Spannen gleich oder geringer 6 mm ist;
Nachlassen der Überdehnungskraft nach dem Spannen, so dass sie 20% der ursprünglichen Überdehnungskraft beträgt oder der für das Stahldrahtseil konzipierten Spannung entspricht; Messen einer Länge des Stahldrahtseils bei einer konstanten Temperatur im Dunklen, und Berechnen einer spannungsfreien Länge des Stahldrahtseils bei einer Referenztemperatur gemäß der folgenden Gleichung: ${L}_{CO} = \frac{{L}_{CP}}{1 + \frac{{P}_{20}}{EA} + α \left(t-{t}_{0}\right)}$ wobei
L_{CO} die spannungsfreie Länge in Metern (m) des Stahldrahtseils bei der Referenztemperatur darstellt;
L_{CP} eine Länge in Metern (m) des mit einer Spannkraft von P₂₀ belasteten Stahldrahtseils darstellt;
P₂₀ 20% der Überdehnungskraft in N darstellt;
A eine nominale Fläche in mm² des nackten Stahldrahtseils darstellt; E ein Elastizitätsmodul in MPa darstellt;
α einen Längenausdehnungskoeffizienten eines Stahldrahtseils darstellt, der gleich 0,000012/°C ist;
t eine stabile Temperatur in °C darstellt, wenn eine Länge des Stahldrahtseils gemessen wird;
und t₀ eine konzipierte Referenztemperatur in °C des Stahldrahtseils darstellt;
bei dem Stahldrahtseil mit dem heiß gegossenen Anker wird an das Stahldrahtseil ein Spitzendruck angelegt, der dem 1,25-fachen der für das Stahldrahtseil konzipierten Spannung entspricht und erfüllt, dass ein Rückzugswert des Gusskörpers innerhalb der Ankerschale nach der Spitzendruckerfassung gleich oder geringer 6 mm ist; und
8) Aufrollen des fertigen umspritzten Stahldrahtseils aus Schritt 7), umfassend
Aufrollen von Schichten des fertigen umspritzten Stahldrahtseils hintereinander unter Verwendung eines Wicklungsrahmens, wobei ein innerer Durchmesser einer erhaltenen Wicklung gleich oder größer als das 20-fache eines Außendurchmessers des Stahldrahtseils und gleich oder größer 1,6 m ist.

2. Verfahren gemäß Anspruch 1, **dadurch gekennzeichnet, dass** wenn die Länge des Standarddrahts in Schritt 2) bestimmt wird, die Spannungskorrektur und Temperaturkorrektur dann gemäß der folgenden Gleichung durchgeführt werden: $L = {L}_{0} \times \left[\left(1+F/EA\right)+α\left(T-20\right)\right]$ wobei
L eine Länge in m des Stahldrahts in einem gespannten Zustand darstellt,
L₀ eine für den Stahldraht konzipierte Länge in m in einem ungespannten Zustand darstellt,
F eine Spannkraft in *N* darstellt,
E ein Elastizitätsmodul in MPa des Stahldrahts darstellt, wobei die Herstellung des Standarddrahts einen gemessenen Wert übernimmt,
A eine Fläche eines Querschnitts in m² des Stahldrahts darstellt, wobei die Herstellung des Standarddrahts einen gemessenen Wert übernimmt,
α einen Ausdehnungskoeffizienten des Stahldrahts darstellt,
und T eine Temperatur der Umgebung darstellt.

3. Verfahren gemäß Anspruch 1, **dadurch gekennzeichnet, dass** eine Außenfläche des doppellagigen Polyethylen-Schutzfilms mit Schneckenlinien oder -prägungen versehen ist, und ein Widerstandsbeiwert gleich oder kleiner 0,8 ist.

4. Verfahren gemäß Anspruch 1, **dadurch gekennzeichnet, dass** Strukturen der Anker in Schritt 6) einen Schraubenmutter-artigen Anker, einen Anker der Art, dass er einen Ankerplattenspalt einstellt, oder einen Haken-Bolzengelenkartigen Anker an beiden Enden des Stahldrahtseils umfassen.

5. Verfahren gemäß Anspruch 1, **dadurch gekennzeichnet, dass** in Schritt 7) ein Fehler in der spannungsfreien Länge des Stahldrahtseils bei der Referenztemperatur die folgenden Bedingungen erfüllt:
wenn L_{CO} ≤ 100 m, beträgt der Fehler weniger oder ist gleich 10 mm; und
wenn L_{CO} > 100 m, beträgt der Fehler weniger oder ist gleich L_{CO}/20000 + 5 mm.

6. Verfahren gemäß Anspruch 1, **dadurch gekennzeichnet, dass** die Umhüllungsbandage eine Bandage aus Polyesterfasern ist; die Umhüllungsbandage eine Breite von zwischen 40 und 60 mm und eine Zugfestigkeit von gleich oder höher als 500 N/25 mm² aufweist.

## Revendications

1. Procédé de fabrication d'un câble en fils d'acier enduit par extrusion, le procédé comprenant les étapes de :
1) fabriquer un fil d'acier comprenant un placage en alliage zinc-aluminium, comprenant :
préparer un placage en alliage zinc-aluminium sur une surface du fil d'acier, dans lequel l'alliage zinc-aluminium est un Zn95Al5 ayant une teneur en aluminium comprise entre 4,2 et 7,2 % en poids ou un Zn90Al10 ayant une teneur en aluminium comprise entre 9,2 et 12,2 % en poids, et un poids du placage en alliage zinc-aluminium est égale ou supérieur à 300 g/m² ;
2) fabriquer un fil d'acier ayant une longueur standard à partir dudit fil obtenu par moyen de l'étape 1), comprenant :
faire d'un fil central un fil standard et déterminer une longueur du fil standard par une mesure de référence, appliquer une certaine force de tension aux deux extrémités d'un fil d'acier pour redresser le fil d'acier et effectuer une correction de tension et une correction de température pour préparer un fil d'acier ayant une longueur standard ; placer certains marqueurs pour couper aux deux extrémités du fil d'acier ; faire du fil d'acier ayant la longueur standard une référence et contrôler une longueur totale du câble en fils d'acier par un procédé de transfert ;
3) tordre un faisceau de fils d'acier pour obtenir un câble en fils d'acier, comprenant :
fournir des fils d'acier obtenus par l'étape 1),
positionner le fil standard dans une position centrale d'une section transversale du câble en fils d'acier à former par une pluralité de couches de fils d'acier ;
tordre tous les fils d'acier dans le faisceau dans la direction gauche avec un angle de torsion α compris entre 2° et 4° et ainsi obtenir un câble en fils d'acier nu ;
et emballer le câble en fils d'acier nu d'un bandage d'enveloppe, dans lequel le bandage d'enveloppe est tordu vers la droite pour obtenir un câble en fils d'acier comme un produit semi-fini ;
dans lequel la longueur L' des fils d'acier à fournir pour ladite pluralité de couches entourant le fil standard est calculée en considérant la longueur du fil standard et l'angle de torsion α selon l'équation suivante : ${L}_{0} = L ′ \times cosa + K ,$ dans laquelle K < 0 dans laquelle
α représente l'angle de torsion ;
K est en mètres (*m*) et est sélectionné selon des spécifications et des opérations ;
L' représente la longueur en mètres (*m*) des fils d'acier à fournir pour les couches entourant le fil standard ;
et L₀ représente la longueur en mètres (*m*) du fil standard à la position centrale ;
4) l'extrusion, comprenant :
préparer un film protecteur en polyéthylène à double couches à l'extérieur du câble en fils d'acier de l'étape 3), dans lequel le film protecteur en polyéthylène à double couches a une densité comprise entre 0,942 et 0,978 g/cm³, une résistance à la fissuration sous contrainte de ≥ 5000 F₀/h et un indice de fusion de ≤ 0,45 g/10 min ; avant l'extrusion, on prédéfinit une ouverture de buse d'une extrudeuse et une vitesse d'extrusion selon un diamètre extérieur du câble en fils d'acier et l'épaisseur des deux couches en polyéthylène ; l'ouverture de buse de l'extrudeuse étant munie de deux couches d'un canal de décharge, et les deux couches en polyéthylène couvrent simultanément le câble en fils d'acier pendant l'extrusion ;
dans lequel un champ magnétique est disposé au-dessus du câble en fils d'acier pour mettre le câble en fils d'acier en un état suspendu ; après le procédé d'extrusion, le film protecteur en polyéthylène à double couches et le câble en fils d'acier nu sont disposés de manière concentrique ;
5) couper, comprenant :
déterminer des positions originales de coupe du câble en fils d'acier enduit par extrusion en retirant localement le film protecteur en polyéthylène à double couches, trouver les marqueurs pour couper aux deux extrémités du fil standard à la position centrale du câble en fils d'acier enduit par extrusion ;
couper le câble en fils d'acier enduit par extrusion en utilisant une machine de découpage non-liquide et assurer des surfaces d'extrémité du câble en fils d'acier enduit par extrusion perpendiculaires à un axe du câble en fils d'acier enduit par extrusion ;
retirer le film protecteur en polyéthylène à double couches selon une longueur prédéfinie pour exposer les fils d'acier ;
6) couler un ancre au câble en fils d'acier enduit par extrusion de l'étape 5), comprenant :
fournir un ancre fonctionnant comme une structure principale de liaison pour transmettre une tension du câble en fils d'acier enduit par extrusion à un pylône ou à une poutre ; comprenant :
effectuer une galvanisation à chaud ou un revêtement de peinture sur l'ancre pour obtenir une résistance à la corrosion, une épaisseur de la galvanisation à chaud étant égale ou supérieure à 90 µm et une épaisseur du revêtement de peinture étant déterminée selon des spécifications et des exigences de conception de la structure en acier ;
couler l'ancre par moyen de coulage à froid d'un ancre de refoulement ou par moyen de coulage à chaud d'un ancre, les opérations s'effectuant comme suivant :
A. coulage à froid d'un ancre de refoulement, comprenant :
a. fixer les extrémités des fils d'acier dans des cupules d'ancrage sur une plateforme de coulée, enlever des tâches d'huile et de rouille des parties des fils d'acier à l'intérieur des cupules d'ancrage et simultanément laver les parois intérieures des cupules d'ancrage ;
b. disperser de manière uniforme les extrémités des fils d'acier selon des trous dans des panneaux d'ancrage et refouler chaque fil d'acier en utilisant une machine de refoulement, les dimensions de refoulement étant les suivantes : diamètre de refoulement ≥ 1,4 D, hauteur de refoulement ≥ 1,0 D et D représente un diamètre des fils d'acier ;
c. fournir et mélanger de manière uniforme un matériau de remplissage refroidi comprenant des boulets en acier, une poussière de pierre, une résine époxy, un agent durcisseur, un di-n-butyle, et un diluant ; verser un mélange du matériau de remplissage refroidi dans les cupules d'ancrage en les faisant vibrer par moyen d'une pompe de vibration pour complètement remplir les fentes entre les cupules d'ancrage et les fils d'acier du mélange du matériau de remplissage refroidi ; ou
B. coulage à chaud d'un ancre, comprenant : fournir un alliage zinc-cuivre comprenant 98 ± 0,2 % en poids de zinc et 2 ± 0,2 % en poids de cuivre, ou un alliage zinc-cuivre-aluminium comprenant 4 - 7 % en poids d'aluminium, 1 - 2 % en poids de cuivre et 91 - 95 % en poids de zinc ; et effectuer le coulage comme suivant :
a. fixer les extrémités des fils d'acier perpendiculairement dans les cupules d'ancrage sur la plateforme de coulée, disperser des fils d'acier comprenant un placage en alliage zinc-aluminium à l'intérieur des cupules d'ancrage en forme des cercles concentriques, enlever des tâches d'huile et de rouille des surfaces des fils d'acier et simultanément laver les parois intérieures des cupules d'ancrage ;
b. maintenir le centre du câble en fils d'acier en coïncidence avec les centres des cupules d'ancrage et empêcher que les fils d'acier touchent aux cupules d'ancrage ;
c. fermer des ouvertures inférieures des cupules d'ancrage pour empêcher que l'alliage s'échappe via les ouvertures inférieures ; et préchauffer les cupules d'ancrage ;
d. verser l'alliage zinc-cuivre ou l'alliage zinc-cuivre-aluminium dans les cupules d'ancrage dans un coulage en une étape en évitant chaque vibration ou interruption ;
7) effectuer une détection de tension ou une détection de pression de tête, comprenant :
selon des matériaux de remplissage pour le coulage de l'ancre, effectuer une détection de tension sur le câble en fils d'acier avec un ancre coulé à froid ou effectuer un détection de pression de tête sur le câble en fils d'acier avec un ancre coulé à chaud avant de quitter l'installation, ce qui se déroule notamment comme suivant :
pour le câble en fils d'acier avec l'ancre coulé à froid, tendre le câble en fils d'acier avec une force grevant, qui est définie entre 1,1 et 1,5 fois une tension conçue pour le câble en fils d'acier et qui satisfait à l'exigence qu'une valeur de rétraction d'un corps de coulée à l'intérieur de la cupule d'ancrage après l'étirement soit égale ou inférieure à 6 mm ;
soulager la force grevant jusqu'à atteindre 20% de la force grevant originale ou jusqu'à atteindre la tension conçue pour le câble en fils d'acier après l'étirement ; mesurer une longueur du câble en fils d'acier à une température constante dans l'obscurité et calculer une longueur sans tension du câble en fils d'acier à une température de référence selon l'équation suivante : ${L}_{CO} = \frac{{L}_{CP}}{1 + \frac{{P}_{20}}{EA} + α \left(t-{t}_{0}\right)}$ dans laquelle :
L_{CO} représente la longueur sans tension en mètres (m) du câble en fils d'acier à la température de référence ;
L_{CP} représente une longueur en mètres (m) du câble en fils d'acier tendu par une force de tension de P₂₀ ;
P₂₀ représente 20% de la force grevant en N ;
A représente une zone nominale en mm² du câble en fils d'acier nu ;
E représente un module élastique en MPa ;
α représente un coefficient de dilatation linéaire d'un câble en fils d'acier, qui est égale à 0,000012/°C ;
t représente une température stable en °C, si on mesure une longueur du câble en fils d'acier ;
et t₀ représente une température de référence conçue pour le câble en fils d'acier en °C ;
pour le câble en fils d'acier avec l'ancre coulé à chaud, appliquer une pression de tête sur le câble en fils d'acier, laquelle pression est 1,25 fois la tension conçue pour le câble en fils d'acier et satisfait à l'exigence qu'une valeur de rétraction d'un corps de coulée à l'intérieur de la cupule d'ancrage après la détection de pression de tête soit égale ou inférieure à 6 mm ; et
8) enrouler le câble en fils d'acier enduit par extrusion fini de l'étape 7), comprenant :
enrouler des couches du câble en fils d'acier enduit par extrusion fini successivement en utilisant un cadre d'enroulement, dans lequel un diamètre intérieur d'une bobine résultant est égale à ou plus grand que 20 fois un diamètre extérieur du câble en fils d'acier et égale à ou plus grand que 1,6 m.

2. Procédé selon la revendication 1, **caractérisé en ce que** si on détermine la longueur du fil standard dans l'étape 2), la correction de tension et la correction de température sont ensuite effectuées selon l'équation suivante : $L = {L}_{0} \times \left[\left(1+F/EA\right)+α\left(T-20\right)\right]$ dans laquelle
L représente une longueur en m du fil d'acier dans un état tendu,
L₀ représente une longueur conçue en m du fil d'acier dans un état non-tendu, F représente une force de tension en *N*,
E représente un module élastique en MPa du fil d'acier, dans lequel on adopte une valeur mesurée pendant la fabrication du fil standard,
A représente une zone d'une section transversale en m² du fil d'acier, dans lequel on adopte une valeur mesurée pendant la fabrication du fil standard,
α représente un coefficient de dilatation du fil d'acier,
et T représente une température de l'environnement.

3. Procédé selon la revendication 1, **caractérisé en ce qu'une** surface extérieure du film protecteur en polyéthylène à double couches est munie de lignes en spirale ou de gaufrages en spirale, et un coefficient de résistance est égale ou inférieur à 0,8.

4. Procédé selon la revendication 1, **caractérisé en ce que** des structures des ancres dans l'étape 6) comprennent un ancre du type de vissage d'écrou, un ancre du type à ajuster une fente de panneau d'ancre, ou un ancre du type d'articulation à tourillon en forme de crochet aux deux extrémités du câble en fils d'acier.

5. Procédé selon la revendication 1, **caractérisé en ce que** dans l'étape 7) une erreur de la longueur sans tension du câble en fils d'acier à la température de référence satisfait aux exigences suivantes :
si L_{C0} ≤ 100 m, l'erreur est inférieure ou égale à 10 mm ; et
si L_{C0} > 100 m, l'erreur est inférieure ou égale à L_{C0}/20000 + 5 mm.

6. Procédé selon la revendication 1, **caractérisé en ce que** le bandage d'enveloppe est un bandage fabriqué en fibres de polyester ; le bandage d'enveloppe a une largeur comprise entre 40 et 60 mm et une résistance à la traction, qui est égale ou supérieure à 500 N/25 mm².
